

## UNITED STATES PATENT OFFICE

2,319,369

## PROCESS OF COLOR PHOTOGRAPHY

Virgil B. Sease, New Brunswick, and John R. Weber, South River, N. J., assignors, by mesne assignments, to E. I. du Pont de Nemours & Company, Wilmington, Del., a corporation of Delaware

No Drawing. Application July 28, 1939,  
Serial No. 287,154

11 Claims. (Cl. 95—2)

This invention relates to color photography and more particularly to methods of producing colored images in multilayer photographic elements. More particularly it relates to novel multilayer photographic elements containing color formers and to a novel process for producing colored images in a multilayer film.

This invention has for an object the preparation of a multilayer photographic film which may be used to record a colored scene or object. A further object is to produce a multilayer film which may be processed in a simple manner to form a color photograph. A still further object is to provide a color printing stock which faithfully and accurately records a colored scene. A still further object is to provide a process for developing and processing multilayer film to produce a color photograph which involves a few simple steps. A still further object is to provide a process for developing and processing an exposed multilayer film to a multilayer, color photograph which can be practiced by the average photographer. Still other objects will appear hereinafter.

Many methods have been suggested for preparing colored photographs, but even the most improved of these, particularly those dealing with superposed multi-layer film requires such a degree of skill and control that the average photographer cannot process his own exposures. Furthermore, the large number of steps involved in processing film by prior art methods renders the cost prohibitive to many photographers. The previous methods of color cinematography involving superposed multilayer film fall into two general classes: (1) those in which the respective photosensitized layers are uniformly colored and the color is discharged differentially with respect to the silver images formed by development. (2) those in which colors are formed step-wise and differentially in respect to the silver images formed by development. Each of these processes is quite involved and requires a great deal of handling of the film. The first-mentioned process known commonly as a "bleach-out" process, depends upon the bleaching-out or removing of dye in direct proportion to the density of the silver in the image. In actual practice it has been difficult to bleach out the dyes entirely in those areas which should be clear of dye. Variations and impurities in the dyes themselves, variations in dyes of the same name or index number but made by different manufacturers, variations in the purity of the chemicals of the bleach-bath and local variations in the rates of

penetration of these baths through the multilayers, have made this process incapable of producing colored photographs on a volume basis.

The second process is even more delicate in its 5 processing requirements since it depends on the controlled diffusion of developers, bleach-baths and stop-baths through thin layers of gelatin. Variations in coating weight, hardness of gelatin, swelling characteristics of the gelatin, temperature of baths, etc., make extremely difficult the 10 volume production of colored photographs by this method.

The above disadvantages are overcome and 15 the objects hereof are obtained by the hereinabove described invention by the use of a novel arrangement of superposed multilayer photographic emulsions and a novel and simplified method of processing.

The novel film is composed of a transparent 20 base having at least two differentially sensitized emulsion layers containing color-formers superimposed thereon, one of the emulsion layers being imposed directly upon the base and being further characterized in that a layer of pre-fogged silver salts is interposed between said 25 emulsion layers.

In the case of three-color photography, two 30 emulsion layers may be placed upon one side of the base and one emulsion layer placed upon the reverse side of the base. In this embodiment of the invention only one pre-fogged silver salt layer is necessary, but two may be employed, one being coated directly on the base. In other embodiments wherein three superimposed layers are on 35 the same side of the base two pre-fogged silver salt layers are employed being placed between the emulsion layers. Color formers as above stated are incorporated in the respective emulsions.

Film suitable for two color photography may 40 consist of a film base having two superposed emulsion layers on one side of the base and a pre-fogged silver salt layer between the sensitized emulsion layers or the emulsion layers may be placed on each side of the base, a pre-fogged layer 45 being between one of them.

The novel film constructions hereof, when used 50 for recording an original scene, can be classified as a negative film and is composed of a series of photo-sensitive silver salt emulsion layers which are individually sensitized to record blue, green and red regions of the spectrum and which contain color-formers which form dyes complementary in color to the utilized region sensitivity of 55 the respective layers. Pre-fogged silver salt layers are interposed between the color sensitive layers.

A yellow filter layer is also embodied in the film so that the red layer will not be exposed to the blue-green end of the spectrum, e. g. green, blue, violet and ultra-violet.

In one important embodiment of the invention the layers are so arranged that light from the scene is first incident on a blue sensitive layer which contains a yellow color-former. A yellow filter dye, e. g. Luxol Fast Yellow T, may be incorporated in the blue sensitive layer or in a sub-layer of gelatine. The light then passes through a pre-fogged emulsion layer, then a green sensitive emulsion layer containing a magenta color-former, then a pre-fogged emulsion layer containing a soluble red dye (e. g. carmosine M), a red sensitive emulsion layer containing a blue-green color former and finally through the base.

The amount of silver-salt in these pre-fogged layers, and the fogging exposure given these emulsion layers is preferably such that upon the first development of the layers a light-barrier layer will be formed in these pre-fogged emulsions so that substantially less than 1% of light will be transmitted by either of them. The present invention thereby provides for an effective control of the printing light penetration by means of the black barrier layers formed from the pre-fogged emulsion layers by the first development step.

In using the film just described, it is exposed normally in a camera, after which it is given a development treatment in a bath containing a non-color-forming developing agent. Any suitable developer which is of the type used as a first developer in a reversal process may be used for this purpose, preferably an energetic-working developer to give full detail and harmonious color rendering. It is also desirable that the developer selected produce a minimum of relief effect in the gelatin. To this end, caustic alkalies should be avoided. Sodium carbonate is preferable as an alkali and is used in smaller amounts than generally used in reversal "first developers." "Metol" in combination with hydroquinone, for instance, is suitable as the developing agent, as are also acid amidol developers. The development at this stage should be carried out completely, that is none of the latent images should be left undeveloped.

After development and washing the film consists of three color separation negative image layers bearing both silver and unexposed undeveloped silver-salt images and two layers of metallic silver in which there may be small amounts of non-color sensitized silver salts. The film is now preferably exposed through the base with a red or white printing light which exposes only the silver-salt image remaining in the red sensitive layer. The printing light does not affect the other two layers because of their lack of sensitivity to the red light, but primarily because the black metallic silver barrier-layer prevents substantially all of the printing light from passing through to other layers.

The film is now developed in a solution containing a color-developing agent, preferably an aromatic diamino developing agent, which will couple with the blue-green to form a dye image in situ with the silver. A suitable developer for this purpose is as follows:

*Developer A*

|                                    |       |      |
|------------------------------------|-------|------|
| Potassium carbonate                | grams | 30   |
| Sodium sulfite, anhydrous          | do    | 5    |
| Diethylamino aniline hydrochloride | do    | 3    |
| Water                              | liter | 1 75 |

This developer forms both silver and blue-green dye images from the exposed silver halides of only the red-sensitive layer. The film is then thoroughly washed.

5 The top or blue sensitive layer is now exposed to a blue or preferably white printing light. The printing light does not have any substantial effect upon the middle or blue-green sensitive layer because of the metallic silver barrier layer between the top and middle layers. The entire film 10 is then treated in a developing solution which contains a developing agent which will couple with the yellow color-former. A suitable developer solution is Developer A. After development the top layer will contain both metallic 15 silver and yellow dye images in situ therewith.

There now remains the green-sensitive middle 20 layer on both sides of which are black, metallic-silver barrier layers. This central layer is preferably chemically exposed by bathing the film in a solution of a mild inorganic reducing agent, e. g. 0.5% aqueous solution of alkaline sodium arsenite or a 5% aqueous solution of hydrogen peroxide. This chemical exposure will make sensitive the silver salts remaining in the middle 25 layer.

As another means of chemical exposure the film 30 may be treated with an aqueous solution of an organic sulfur-bearing compound such as a 5% aqueous solution of guanidine thiocyanate or guanyl thiourea, thiourea, allyl thiourea, imino amino sulfonic acid of a pH of at least about 7.1.

35 It is not necessary, however, to resort to chemical exposure of the middle layer to render it exposed or so that the silver salts are sensitized. Thus, the middle layer may be exposed by means of X-ray exposure of the entire film, or by means of mechanical vibrations of a class known as "ultrasonic" vibrations. In the latter case the entire film, during the latter part of the washing operation following the yellow development, may be subjected to ultrasonic vibrations, or the film, after washing may be immersed in water or some non-film solvent and then subjected to ultrasonic vibrations. The central layer can also be exposed by means of heat rays, in which case the entire film should be immersed in 5% formaldehyde solution before exposing to the heat rays.

After the middle layer has been exposed, the 40 entire film is treated or developed in a solution containing a developing agent which will couple with the magenta or minus-green color former to form a magenta dye upon development. A suitable developer is Developer A above described.

50 After this final development, the silver is removed from all the layers by means of a photographic reducing bath. Any of the conventional reducing baths may be used at this stage of the process. Suitable baths include Farmers Reducer and permanganate, sulfuric acid. The former may be used either as a combined bath or separately, by immersing the film in a 5% solution of potassium ferricyanide and then in a 20-40% sodium thiosulfate solution. The sulfamic acid bleach bath of McQueen and Goebel application, Serial No. 233,117, filed October 3, 1938 now U. S. Patent 2,195,419, may also be used.

55 In a modification of the invention which is of considerable importance a green blind red-sensitive layer occupies the central position of the multilayer film. This green-blind red sensitive layer is sensitized by means of pinacyanol or one of the naphthoseleno carbocyanines such as sym-

3:3' - diethyl-naphthoselenocarbocyanine iodide described in co-pending application No. 78,734, filed May 8, 1936, or the green blind sensitizing dyes described in U. S. Patents 2,148,979, 2,148,980, and Piggott and Rodd U. S. Patent 2,071,898. The sym-3:3' - diethyl-naphthoselenocarbocyanine iodide was prepared by reacting one part of 2-methyl-alpha-naphthoseleno ethiodide with one part of ethyl-ortho-formate in the presence of 6 parts of dry pyridine by heating the admixture under reflux for 20 minutes. The 2-methyl-alpha-naphthoseleno ethiodide was prepared by reacting 2-methyl-alpha-naphthoselenazole with three mols of ethyl iodide under reflux for 24 hours, evaporation of the excess ethyl iodide and crystallization of the product from alcohol.

The base was made in the following manner:

A solution of 51 parts of the hydrochloride of 1-bromo-2-aminonaphthalene in about 70 parts of alcohol was treated with 28 parts of potassium selenocyanate in 80 parts of water. After standing over night at room temperature, the mixture was evaporated to dryness and extracted many times with hot water. The extract was made alkaline with ammonia and the aminonaphthoselenazole precipitated. It was recrystallized from alcohol. Yield 36 parts; M. P. 252° C. This compound has the formula:



A mixture of 28 parts of the aminonaphthoselenazole, 28 parts of sodium hydroxide and 50 parts of water was heated together in an nickel crucible for three hours on an electric hot plate. The cover of the crucible was adjusted so that steam could escape. Water lost by evaporation was replaced as it boiled off. Finally the crucible was evaporated to dryness and heated until the fumes due to decomposition began to appear. The residue was taken up with water and filtered. The filtrate was cooled, and dilute hydrogen peroxide added drop by drop until no more precipitation formed. The precipitated diselenide, a yellow amorphous powder, was separated by filtration, washed and dried. A yield of 13 parts was obtained. This compound has the formula:



This was heated to boiling in 108 parts of acetic anhydride under a reflux condenser and 4 parts of zinc gradually added. Heating was continued for thirty minutes. The hot solution was filtered from some unreacted zinc, and poured into water. The solution was later extracted with ether, and after drying the ether solution and removing the ether by evaporation, needle crystals of the 2-methyl-alpha-naphthoselenazole were obtained. It melted at 81-82° C. Yield 7 parts.

In a manner similar to that just described, other 2-methyl-naphthoselenazoles and their quaternary salts may be prepared. The naph-

thalene nucleus, for instance, may contain methyl, ethyl, or propyl methoxy or ethoxy radicals in one or more of the 3-, 4-, 5-, 6-, 7-, or 8-positions. The quaternary salts may be condensed to form cyanine dyes in like manner. The multilayer film used in this modification consists of a support coated on one side with a green sensitive emulsion containing a magenta color former, then a pre-fogged layer on which is coated a green-blind red-sensitive emulsion containing a blue-green color former on which is coated a blue-sensitive emulsion containing a yellow color-former. The last mentioned layer may contain yellow filtering agent, e. g. titanium ferrocyanide, or the yellow filter may be incorporated in a separate gelatin sub-layer.

In using the just described film, it is exposed normally in a camera with the emulsion facing the lens. It is then processed to colored positives by the following steps:

1. Develop in a non-color forming developer, e. g. of the type hereinbefore described;

2. After washing, the film is flashed through the base with white or green light which exposes the green sensitive layer but not the red or blue layers due to the barrier layer of metallic silver formed by the first development;

3. The film is then developed in a solution containing a developing agent capable of coupling under the development conditions with the magenta color-former to form a magenta dye image and metallic silver in situ therewith;

4. The film is washed thoroughly and then flashed to orange-red light which exposes the central layer;

5. The film is now developed after the manner of step 3 to form a blue-green color dyed image and metallic silver;

6. The film is washed thoroughly to remove developer etc. and the outer layer is flashed by means of white light which exposes the blue-sensitive layer;

7. The film is now developed after the manner of step 3 to form a yellow dyed image and metallic silver;

8. After washing the silver deposits in the emulsion and barrier layers are removed by means of a reducing agent such as Farmer's Reducer or by treatment with cupric bromide, followed by a clearing bath of hypo and a final wash.

A film similar to that just described but which has the green sensitive layer on one side of the base and the green-blind, red sensitive, and blue sensitive layers mounted upon the opposite side is made. In this modification a pre-fogged layer is placed between the green-sensitive layer and the base, but no pre-fogged layers are placed upon the other side between the green blind and blue sensitive emulsion layer. This type of film contains the same type of color-formers and may be processed in the same manner as the immediately preceding type.

Another film construction which can be processed by the processes hereof comprises a film base having a pre-fogged layer, preferably containing a red dye, on one side of a transparent film base over which is coated a red sensitive

layer containing a blue-green color-former, on the other side of the base is first a green sensitive layer containing a magenta color former, next a pre-fogged silver halide layer, and finally, a blue sensitive layer containing a yellow color former. This film may be processed in

the manner first described for the film of the first example.

The invention, however, is not limited to three color photography, but on the contrary, can be used with two color photography, wherein a pre-fogged layer is placed between two differentially sensitized emulsion layers containing color formers, either directly or indirectly by reason of one layer being disposed upon the opposite side of a film base.

A film similar to that used in the preceding modifications is employed for the multi-color positive prints. In this modification, three color-separation negatives are required. These may be made in a camera or from a colored transparency or from a colored reflection print or by reflection copying. Positive prints in black and white may be made from these negatives or the negatives themselves may be reversed into positive records. Three positive separation records are printed onto the multi-layer film previously described. The sequence of printing operations is not important but the following serves as being illustrative of a preferred procedure:

(a) The blue record positive is printed by white or blue light onto the top layer;

(b) Red record positive is printed by orange red light, through the top layer onto the central layer;

(c) The green record positive is printed by green or white light, through the base onto the bottom layer;

(d) The film is developed in an ordinary non-color-forming developer, such as the "first" developer of a reversal process and the film is processed to color by following through the steps two to eight inclusive as described in the preceding modification. There are a great many color-formers which can be used in the processes described herein and it is to be distinctly understood that the invention is not limited to any particular class or classes. They are preferably non-migratory.

As examples of suitable non-migratory yellow color-formers which may be used in the blue-sensitive layer, mention is made of the diacylacet-amino-aryl-bis-thiazoles of U. S. Patent 2,140,540, of which difuroylacetamino-1,2,4,5-benzo-bis-thiazole and di-acetoacetamino-1,2,4,5-benzo-bis-thiazole are especially useful as are 2-hydroxy-3-naphthoylaminobenzoyl-acetanilide, sodium stearoylaminobenzoylacetanilide-p-carboxylate, p-caproylaminobenzoylaminosalicylic acid, furoylacet-p-amino phenyl-ethyl ether (described in Jennings and Middleton application, Serial No. 215,702, filed June 24, 1938, now U. S. Patent 2,184,303), and di-picolinoyl-acet benzidine.

Suitable non-migratory magenta color-formers which are especially useful are 1-(3'-sulfo-phenyl)-3-(4'-stearoyl-amino phenyl)-5-pyrazolone sodium salt, 1-(4'-oxy-3'-carboxyphenyl)-3-(4'-dodecoylaminophenyl)-5-pyrazolone, 4,4'-di-(carboxyl-1-p-aminophenyl-3-methyl-5-pyrazolone), 4,4'-bis-(3'-methyl pyrazolonyl-1')-diphenyl (described in Jennings and Middleton, Serial No. 215,703, filed June 24, 1938, now U. S. Patent 2,200,924), 4,4'-methylene-bis-(m-stearoylaminophenyl)-methyl pyrazolone (described in Jennings, Serial No. 256,201, filed February 13, 1939, now U. S. Patent 2,294,909), and 4,4'-o-sulfo-benzylidene-bis-(phenyl methyl pyrazolone) (described in Jen-

nings, Serial No. 256,201, filed February 13, 1939, now U. S. Patent 2,294,909).

Suitable non-migratory blue-green color formers of especial utility include 4,4'-di-(1-hydroxy-

- 5 2-naphthoylaminophenyl), diphenyl, 1-hydroxy-2-carboxy-5-dodecoylaminophenyl, naphthalene, 1-N-stearoyl-4-N-(1'-oxy-2'-naphthoyl)-phenyl-enediamine sodium sulfonate, resorcinol mono-n-dodecyl ether (described in Salzberg and White, 10 Serial No. 164,984, filed September 21, 1937, now U. S. Patent 2,166,181), product of p-hydroxybenzoic acid and formaldehyde (described in McQueen, Serial No. 261,794, filed March 14, 1939), 15 product of polyvinyl alcohol and salicylaldehyde (described in Dorough and McQueen, Serial No. 233,480, filed October 5, 1938, now United States Patent 2,310,943).

There are a large number of developing agents which may be used in the second color development step of the process. The developers are aromatic amino compounds and may contain a plurality of amino groups or substituted amino groups and/or hydroxy groups. They must, however, contain at least one unsubstituted amino group (-NH<sub>2</sub>).

The preferred developing agents in the process of dye coupling development are derivatives of p-phenylenediamine and particularly the asymmetric dialkyl p-phenylenediamines, e. g. p-30 aminodimethylaniline, p-aminodiethylaniline, p-aminodibutylaniline, etc. Other developing agents which may be used include p-phenylenediamine itself, p-methylaminobenzene, p-ethylaminobenzene, p-aminophenol, N,N-diethyl-o-phenylene-diamine, chloro-p-phenylenediamine, 1,2,5-toluylenediamine, 2-amino-5-diethylamino-toluene, N-p-aminophenylpiperidine, N-methyl-N-hydroxyethyl-p-phenylenediamine, N-butyl-N-hydroxyethyl-p-phenylenediamine,  $\beta$ - $\gamma$ -dihydroxy-propyl-p-phenylenediamine, 2-amino-5-(N- $\beta$ -hydroxy-ethyl-N-butyl) aminotoluene and its dihydrochloride, etc. These aromatic amino-developing agents may be used in the form of their salts, which may be either inorganic or organic. The salts are in general more stable than the free bases. As examples of suitable salts mention is made of the hydrochloride, sulfates, acetates, etc.

50 The novel film constructions of the present invention containing color-formers in the emulsion layers have a number of advantages over the film of our co-pending application, Serial No. 121,904, now U. S. Patent 2,191,502, of which this application is a continuation-in-part. These advantages will be apparent from the following description.

(1) The rates of coupling are different for different color-formers. Inasmuch as, for a given time of development, the amount of dye formed is proportional, (but not necessarily equivalent to), the rate of coupling and the amount of development, and since the amount of development is functional with the amount of silver halides exposed, the barrier layers of metallic silver allow the outer emulsions to be controlled-exposed by the second exposure of the reversal process in accordance with the dye-forming characteristics of the individual layer.

In order to determine the amount of second exposure, a test strip of film, given a very slight over-all exposure to white light, is processed through by any of the above-described methods. The processed film should, if the dye-coupling

balance is correct, produce an overall neutral gray density. If the dye-coupling rate is off-balance in one of the layers, the film will show a decided color and will not be neutral gray. Thus, if the yellow color-forming layer is too slow in its dye-forming, the resulting film will be bluish; if the blue-green layer is slow, the film will be reddish; if the middle one is slow it will be greenish. If the chemical exposure has been too light, the final film will be greenish. Thus, by means of this slightly-flashed test strip on the raw stock (which may be an unexposed end of the roll or a piece of the cut film), the dye-forming characteristics of the emulsion are predetermined and the amount of second exposure, both chemical and light, are determined in accordance with the dye-forming characteristics of the individual emulsion layers.

(2) The different color-formers have different effects on the emulsions. Some color-formers sensitize and fog the emulsion layers, thus producing more dye density than ordinarily. Others may decrease emulsion speed thus yielding less dye density than should be expected. By controlling the amount of second exposure, these variations in emulsion characteristics, (and thus variations in dye-densities), can be compensated for by first determining the dye-forming characteristics of the film as described above.

(3) Lack of uniformity from batch-to-batch of color-former likewise causes variations in the characteristics of the final dye images. These variations are compensated for in a similar manner as described above. Thus, the present invention includes the method of processing such fogged barrier layer films by varying the second exposure in accordance with the dye-generating characteristics of the individual emulsion layers.

As many apparently different embodiments of this invention may be made without departing from the spirit and scope thereof, it is to be understood that we do not limit ourselves to the specific embodiments herein except as defined by the appended claims.

We claim:

1. A photographic element comprising a transparent base having at least two differentially sensitized emulsion layers each containing a non-migratory color former capable of forming a dye by color coupling development superimposed thereon the color formers of the respective layers being capable of forming a dye different in color from that formed in the other layers, one of said layers being imposed directly upon the base and a layer of pre-fogged silver salts interposed between said emulsion layers.

2. A photographic element comprising a transparent base having at least two differentially sensitized emulsion layers containing non-migratory color-formers superimposed thereon, one of said layers being imposed directly upon the base and a layer of pre-fogged silver salts interposed between said emulsion layers, the color-formers in the respective layers forming dyes upon development which are complementary in color to the color sensitivity of the respective emulsion layers.

3. A photographic element comprising a transparent base having at least three differentially sensitized emulsion layers superimposed thereon, each containing a non-migratory color former capable of forming a dye by color coupling development, the color formers of the respective layers being capable of forming a dye different in color from that formed in the other layers, one

of each of said layers being imposed directly upon the base and a layer of pre-fogged silver salts interposed between each of said emulsion layers.

4. A photographic element comprising a transparent base having three emulsion layers sensitized red, green and blue, respectively, superposed thereon, the red layer being imposed directly on the base, a non-migratory color-former in each of said emulsion layers capable of yielding a dye complementary in color to the sensitivity of the respective layers upon color coupling development, a pre-fogged silver salt layer interposed between each of the emulsion layers.

5. A film element comprising a transparent base, a red-sensitive emulsion layer containing a non-migratory blue-green color-former imposed directly on said base, a pre-fogged silver salt layer imposed on said red layer, a green-sensitive layer containing a non-migratory magenta color-former imposed on said pre-fogged layer, a pre-fogged silver salt layer, and finally a blue sensitive layer containing a non-migratory yellow color former.

6. A film element of the type set forth in claim 5, wherein a yellow filter layer is positioned in front of the red sensitive layer.

7. A film element comprising a transparent base, a green-sensitive emulsion layer containing a non-migratory magenta color-former imposed directly on the base, a pre-fogged silver salt layer imposed on said green sensitive layer, a green-blind panchromatic layer containing a non-migratory blue-green color former, a blue-sensitive emulsion layer containing a non-migratory yellow color former imposed on said panchromatic layer.

8. A photographic element as set forth in claim 7, wherein a yellow filter layer is positioned in front of said panchromatic layer.

9. The process for forming a multicolor picture on the photographic element of claim 1, which comprises exposing said element to form color separation records of an object, developing therein partial images of said object in a non-color forming developer, re-exposing the remaining sensitive salts in the outer sensitive layer, developing the said sensitive layer in with an aromatic amino developing agent having an unsubstituted amino group, re-exposing the salts remaining in the other sensitive layer and developing the layer with an aromatic amino developing agent having an unsubstituted amino group and removing all silver formed by the foregoing steps.

10. A process for forming a multicolor picture in the photographic element of claim 3, which comprises exposing said element to form color separation records of an object, developing therein the partial images of said object, re-exposing the remaining sensitive salts in the two outer layers by respectively exposing them to light having the same wave lengths as that to which the respective emulsion layers are sensitive and developing said layers with an aromatic amino developing agent having an unsubstituted amino group, chemically exposing the middle layer, developing said layer with an aromatic amino developing agent having an unsubstituted amino group and removing all silver formed by the foregoing steps.

11. A process for forming multi-color pictures which comprises developing an exposed test strip of a film element of the type set forth in claim 3, developing the strip in a non-color forming developer, re-exposing the remaining salts in one

of the outer sensitive layers and developing said layer with an aromatic amino developing agent having an unsubstituted amino group, re-exposing the salts remaining in the other outer sensitive layer and developing said layer with an aromatic amino developing agent having an unsubstituted amino group, chemically exposing the middle layer and developing the same with an

5 aromatic amino developing agent having an unsubstituted amino group; removing all silver formed by the foregoing steps; and regulating the processing of the film element in accordance with the dye-forming characteristics of the individual emulsion layers.

VIRGIL B. SEASE.  
JOHN R. WEBER.